

Patented Sept. 2, 1952

2,609,309

# UNITED STATES PATENT OFFICE

2,609,309

## MAGNESIUM ALLOY AND METHOD OF TREATMENT

Jerzy W. Meier, Ottawa, Ontario, Canada, assignor to Her Majesty the Queen in the right of Canada as represented by the Minister of Mines and Technical Surveys

No Drawing. Application January 22, 1949, Serial No. 72,260. In Canada October 7, 1948.

2 Claims. (Cl. 148—21.90)

1

This invention relates to magnesium casting alloys and a method of treating the same and more particularly to a magnesium casting alloy containing both zinc and zirconium.

Zirconium has been classified among metals which have the capacity to harden alloys. It is known to have the property of reducing the grain-size of magnesium alloys. Zinc has been used in magnesium alloys.

The object of the present invention is to provide an alloy which has a maximum ratio of strength to weight in order to best adapt it for use in airborne and transportation equipment where weight is a major consideration.

A further object of the invention is to provide an improved method of treating magnesium alloys containing zirconium.

The alloy of the invention in its preferred form contains 6% of zinc and not less than 0.7 nor more than 1 per cent of zirconium in magnesium. In producing such alloy it is rather difficult to closely control the precise proportions of minor components in the finished alloy. In accordance with the present invention, in no case should the zinc exceed 7 per cent nor be less than 5 per cent. It is desirable that the zinc content be not allowed to vary from the preferred 6 per cent by more than 0.5 per cent. Less than 0.7 per cent of zirconium has been found to give markedly inferior results in the grain-size of the alloy and in the effectiveness of the ageing or heat treatment in developing maximum strength and ductility in the alloy.

It is believed by those skilled in the art of producing zirconium-containing magnesium alloys that it is zirconium, which is in solid solution, that effects the grain size of the alloy. It is also known that very careful foundry technique is essential to insure high effective zirconium content in solid solution. When carefully prepared accordingly the present alloy has an average grain diameter of 0.001 to 0.002", in no case exceeding 0.003", and the following average mechanical strength properties:

Ultimate tensile strength, 38,000—42,000 p. s. i.  
Yield strength, 18,000—22,000 p. s. i.

Elongation, 8 to 14%

A comparison of this alloy, in the "as cast" condition, i. e. without heat treatment, with similar alloys containing a smaller proportion of zinc shows that the present alloy has much superior mechanical properties. This is illustrated by an increase of as much as 13 per cent in ultimate tensile strength, 15 per cent in yield strength and

more than 30 per cent in elongation found in many test bars of the alloy.

A similar comparison of such alloys after heat treatment showed an increase of as much as 30 per cent in ultimate tensile strength, 50 per cent in yield strength and in elongation in bars tested.

An important characteristic of the alloy is that its mechanical properties of strength and hardness are developed by ageing at room temperature to a greater extent than in similar alloys.

It has been found that the effect of heat treatment on magnesium alloys containing zirconium, with or without other metals, in the development of maximum desirable mechanical properties, i. e., strength and ductility, is much improved by subjecting them to a homogenizing treatment at a high temperature and to an ageing treatment at a low temperature.

In accordance with the method of the invention, the cast alloys are subjected to a homogenizing treatment at a temperature of at least 425° C. for a short period which should not exceed five hours and to an ageing treatment at a temperature not exceeding 150° C. For the first stage of the heat treatment the preferred temperature is 475 to 500° C. and heating at such temperature for a period of one half hour is effective. A two hour period is preferred. At lower temperatures a somewhat longer period is preferred but this temperature should not be less than 425° C. In the second or ageing stage of the method the alloy is maintained at a temperature not exceeding 150° C. for at least 24 hours, preferably 48 hours.

To illustrate the effect of this treatment the following example is given:

An alloy containing magnesium and 5.88 per cent zinc and 0.82 per cent zirconium in the "as cast" condition had an ultimate tensile strength of 39,100 pounds per square inch, a yield strength of 20,800 p. s. i. and an elongation of 10.1 per cent. When this cast alloy was heat treated as above described, the comparative figures were respectively 47,300, 30,700 and 14.

45 What is claimed is:

1. A method of developing strength and ductility in magnesium casting alloys consisting essentially of magnesium, substantially 6% zinc and not less than 0.7 nor more than 1% zirconium which comprises subjecting the cast alloy to a homogenizing treatment at a temperature of 425 to 500° C. for a relatively short period of time not exceeding 5 hours but sufficient to effect optimum homogeneity of the structure at the particular temperature employed and thereafter to an age-

ing treatment at a temperature not exceeding 150° C. for at least 24 hours and sufficient to develop in the casting an ultimate tensile strength not less than 42,000 p. s. i., and a yield strength substantially greater than 25,300 p. s. i.

2. An alloy casting as and when produced by the method defined in claim 1.

JERZY W. MEIER.

REFERENCES CITED

The following references are of record in the file of this patent:

UNITED STATES PATENTS

| Number    | Name        | Date          |
|-----------|-------------|---------------|
| 1,936,550 | Gann et al. | Nov. 21, 1933 |
| 1,985,421 | Paine       | Dec. 25, 1934 |

| Number      | Name        | Date          |
|-------------|-------------|---------------|
| 2,224,151   | Gauthier    | Dec. 10, 1940 |
| 2,286,311   | Sauerwald   | June 16, 1942 |
| 2,314,853   | Brandt      | Mar. 23, 1943 |
| 5 2,420,293 | Beck et al. | May 13, 1947  |
| 2,520,753   | Ball et al. | Aug. 29, 1950 |

FOREIGN PATENTS

| Number     | Country | Date          |
|------------|---------|---------------|
| 10 211,152 | France  | Nov. 18, 1940 |

OTHER REFERENCES

Serial No. 369,749, Sauerwald et al. (A. P. G.), published June 15, 1943.

15 Doan et al.: Treatise in Transactions, American Institute of Mining and Met. Engrs., vol. 171, 1947, pages 286-305.